

Sept. 13, 1932.

J. N. GOLDSMITH

1,877,658

COLOR PHOTOGRAPHY

Filed May 22, 1930

Fig. 1.



Fig. 2.



Fig. 3.



Fig. 4.



RED



GREEN



VIOLET

INVENTOR

J. N. Goldsmith,  
By Watson, Dot  
Morse & Knudle  
ATTYS

## UNITED STATES PATENT OFFICE

JOHN NAISH GOLDSMITH, OF LONDON, ENGLAND, ASSIGNOR TO SPICERS LIMITED, OF LONDON, ENGLAND, A BRITISH COMPANY

## COLOR PHOTOGRAPHY

Application filed May 22, 1930, Serial No. 454,833, and in Great Britain May 30, 1929.

This invention comprises improvements in or relating to color photography, and relates especially to methods for the application of a multicolor screen to a film comprising celluloid, or a cellulose ester, such for example as cellulose acetate or nitro-cellulose. These films are herein referred to collectively as cellulose ester base films. The instant process is applicable in those processes of the type in which there is applied to the surface of the film at one or more stages of the process a series of lines or other geometrical patterns of a greasy resist-material, i. e. a material capable of protecting the underlying portions of the film from solutions of dyes or bleaching agents. Thus, for example, oily resists may be employed to protect the film from aqueous or aqueous alcoholic dye solutions.

One example of a process of this general type is given in British Patent No. 322,432, according to which the film dyed uniformly with one color (say green) is led through a printing machine by means of which extremely fine parallel lines of greasy ink (intended to act subsequently as fatty resists) are printed upon it. The printing is effected by means of a small engraved steel roller having, for example, fifteen lines and fifteen intervening grooves per millimeter. When the ink is dry the film is passed into contact with a bath which bleaches and dissolves out the green dye from the spaces between the lines, leaving unattacked the green lines protected by the ink. Thereafter the film has applied to it another dye, say a red dye, which colors only the spaces between the ink lines, and so forth.

It is one object of the present invention to provide means whereby, in processes of the above described type, the steps of covering the whole surface of the film with one dye, and subsequently bleaching the dye from the inter-spaces between the first series of the

resist pattern, may be avoided. In effect when the film has received the lines of resist-medium embodying one dye and when the film has been suitably dried, it may be immediately treated with the next color to produce colored lines between the first mentioned lines.

According to the invention in a method of the type described for applying a multi-color screen for color photography to a film comprising celluloid, or a cellulose ester, the resist-medium employed to print one or more of the series of lines or other geometrical pattern upon the film, contains a dye which penetrates from the medium into the film, so that on removal of the medium, for example by washing with a solvent, a geometrical pattern in color remains on the film.

In the drawing, Fig. 1 shows a film coated with a dye containing resist.

Fig. 2 shows the film after dyeing between the lines of resist and removing the resist.

Figs. 3 and 4 show a three color variation. According to a feature of the invention, the dye-bearing medium may comprise a fatty or greasy ink, which is printed on the film in a series of lines, so that after removal of the ink (by washing with benzene) a series of colored lines remains on the film.

The dye-bearing medium may comprise a resist, a dye miscible with or soluble in said resist and an agent (such as acetic acid) which is a solvent for the dye and enables the dye to penetrate into the surface of the film.

The dye-bearing medium may alternatively comprise a resist consisting of thickened linseed oil or like thickened vegetable oil, an oil-soluble dye such as "oil orange" or "oil red", and acetic acid. Any of the dyes in the groups known as "oil orange" and "oil red" may be employed, for instance, those defined under these headings in the color index of the Society of Dyers and Colorists, edited by F. M. Rowey, published in 1924 and sup-

plemented in 1928, and the difference between the spectral absorptions of the various dyes may be compensated for where necessary in the manner known to those skilled in the art.

6 The specific color value of the dye used is thus of no great importance, it being desirable, however, that the dyes selected should be soluble in oil and insoluble in water.

According to a particular form of this invention, after lines of a resist-material embodying a dyestuff have been printed on the film, a dyestuff of a different color is applied to those portions of the film which are unprotected by the resist-lines so that after removal of the resist-lines a series of parallel lines in alternate colors is then left on the film.

The invention will now be described with reference to the accompanying drawing, 20 which, it is to be understood, is diagrammatic only.

The surface of a cellulose ester film is first covered with a series of parallel lines *a* of a resist material containing dye, see Fig. 1.

25 An example of a suitable resist material is as follows:

|                       | Grams |
|-----------------------|-------|
| Oil red               | 20    |
| Thickened linseed oil | 20    |
| 30 Acetic acid        | 20    |

The surface of the film is then submitted to the action of a green dye bath, e. g. malachite green. The dye will only affect the portions of the film *b* which are unprotected by the resist lines. The red dye contained in the resist material will, however, penetrate from the resist into the underlying portions of the film, so that on removing the resists the film will be found to be dyed in a series 40 of parallel green and red bands *c* and *d* as illustrated in Fig. 2.

If it is desired to obtain a three color screen on the film, a second series of resist lines *e* which, however, contains no dye, is ruled on 45 the film at right angles to the first series of lines, as shown in Fig. 3. The color is then bleached from the portions of the film between the resist lines, and these portions are then dyed violet.

50 On removing the resists, a three color screen is obtained comprising, as shown in Figure 4, a series of parallel violet lines separated by bands consisting of alternate green and red squares.

55 I claim:

1. A method of the type described for applying a multi-color screen for color photography to a cellulose ester base film wherein the resist-medium employed to print one or more 60 series of lines or other geometrical patterns on the film, contains a dye which penetrates into the medium of the film, so that on removal of the medium a geometrical pattern in color remains on the film.

65 2. A method according to claim 1 where-

in the dye-bearing medium comprises a fatty or greasy ink, which is printed on the film in a series of lines, so that after removal of the ink a series of colored lines remains on the film.

3. A method according to claim 1 wherein the dye-bearing medium comprises a resist, a dye miscible with or soluble in said resist and an agent which is a solvent for the dye and enables the dye to penetrate into the 75 surface of the film.

4. A method according to claim 1 wherein the dye-bearing medium comprises a resist consisting of thickened vegetable oil, an oil-soluble dye selected from the groups consisting of "oil orange" and "oil red" dyes and acetic acid.

5. A method according to claim 1 wherein the dye-bearing medium comprises a fatty or greasy ink, which is printed on the film 85 in a series of lines, so that after removal of the ink by washing with benzene, a series of colored lines remains on the film.

6. A method according to claim 1 wherein the dye-bearing medium comprises a resist, 90 a dye miscible with or soluble in said resist and acetic acid.

7. A method of the type described for applying a multi-color screen for color photography to a film containing a cellulose ester, 95 wherein the resist-medium employed to print one or more series of lines or other geometrical patterns on the film, contains a dye which penetrates from the medium into the film, so that on removal of the medium a geometrical 100 pattern in color remains on the film, and wherein after lines of a resist-material embodying a dyestuff have been printed on the film, a dye-stuff of a different color is applied to those portions of the film which are unprotected by the resist lines so that after removal of the resist lines a series of parallel 105 lines in alternate colors is left on the film.

8. In a process of the nature described of applying a multi-color screen to a cellulose ester base film, the step comprising applying to said film a resist-medium containing a dye in solution capable of penetrating from said resist into said film, and subsequently removing said resist medium, leaving said 110 dye on said film.

9. In a process of the nature described of applying a multi-color screen to a cellulose ester film, the step comprising printing on said film in at least one series of lines a resist-medium containing a fatty or greasy ink and dye and subsequently removing said resist medium, leaving said dye on said film.

10. In a process of the nature described of applying a multi-color screen to a cellulose ester film, the step comprising applying to said film a resist-medium composed of a resist, a dye miscible with said resist and a mutual solvent for said dye and said film,

70

80

85

90

95

100

105

110

115

120

125

130

whereby said dye aided by said solvent penetrates into said film.

11. The method according to claim 8 wherein the resist-medium is composed of a thickened vegetable oil, an oil-soluble dye and a solvent for said dye.

12. The method according to claim 8 wherein the resist-medium is composed of thickened linseed oil, an oil-soluble dye and a solvent for said dye.

13. The method according to claim 8 wherein the resist-medium is composed of thickened linseed oil, an oil-soluble dye and acetic acid.

14. A process of applying a multi-color screen to a cellulose ester film adapted for color photography comprising printing on said film at least one series of lines of a resist-medium containing a dye miscible therewith and capable of penetrating the film, applying a dyestuff of a different color to those portions of the film not protected by the resist lines and removing the resist lines, whereby a film is produced containing a geometrical design of alternate series of lines of dyes of different colors.

15. The process according to claim 14 wherein the resist-medium is a fatty or greasy ink having a dye dissolved therein.

16. The process according to claim 14 wherein the resist-medium is a fatty or greasy ink containing an oil soluble dye and acetic acid.

17. A process of applying a multi-color screen to a cellulose ester film adapted for color photography comprising, printing on said film a series of lines of a thickened linseed oil resist containing acetic acid and an oil dye selected from the groups consisting of oil red and oil orange dyes, drying said resist, applying a dyestuff of a different color to those portions of the film which are unprotected by the resist lines, and removing the resist lines by dissolving the same with benzene, whereby there remains alternate lines of different colors, the dye in said resist having penetrated into the film.

18. A method of the type described for applying a multi-color screen for color photography to a cellulose ester base film wherein the resist-medium employed to print one or more series of lines or other geometrical patterns on the film, contains a dye which penetrates from the medium into the film, so that on removal of the medium by washing with a solvent a geometrical pattern in color remains on the film.

19. A method of the type described for applying a multi-color screen for color photography to a film containing a cellulose ester, wherein the resist-medium employed to print one or more series of lines or other geometrical patterns on the film, contains a dye which penetrates from the medium into the film, so that on removal of the medium by washing

with a solvent a geometrical pattern in color remains on the film, and wherein after lines of a resist-material embodying a dyestuff have been printed on the film, a dyestuff of a different color is applied to those portions of the film which are unprotected by the resist lines so that after removal of the resist lines a series of parallel lines in alternate colors is left on the film.

In testimony whereof I affix my signature.

JOHN NAISH GOLDSMITH.

80

85

90

95

100

105

110

115

120

125

130